

1

2,751,360

## PRESOLVATED ALUMINUM SOAP GELLING AGENTS

Richard E. Van Strien, Griffith, Ind., assignor to Standard Oil Company, Chicago, Ill., a corporation of Indiana

No Drawing. Application December 30, 1953,  
Serial No. 401,397

10 Claims. (Cl. 252—316)

This invention relates to improvements in the preparation and use of bodying agents for liquid hydrocarbons. More particularly, the invention pertains to improved gelling agents capable of gelling liquid hydrocarbons at a rapid gelation rate to obtain stable gels for use as military incendiaries.

Specifically, the invention is directed to the preparation and use of a bodying agent adapted to form, at relatively low bodying agent concentration, stable gels of relatively high consistency with a wide boiling range of petroleum gasolines, jet fuels, diesel fuels and kerosenes, preferably liquid hydrocarbons boiling within the range of from about 100° to 600° F. Such solidified or gelled liquids are useful as charges for incendiary bombs, grenades, flame throwers, and the like.

Exacting requirements for military incendiary gelling agents have been established. Hydrocarbon gels made therefrom must be stable at temperatures over the range of from about -40° to +65° C., so that they may be used in any climate. They must not be susceptible to premature breakdown with loss of viscosity. They must adhere to a target sufficiently long to set it on fire. They must be capable of easy ignition even at subzero temperatures. In addition, it is highly desirable that the gelling agent be capable of forming gels which meet these requirements with a wide variety of hydrocarbon fuels at a rapid rate of gelation and at the lowest possible concentration for purpose of economy of material as well as economy of time and storage space necessarily limited under wartime conditions. In general, most gelling agents for hydrocarbon fuels have not met all of the above requirements. Gelling agents which have the property of imparting high rates of gelation to liquid hydrocarbons at relatively low concentrations in hydrocarbon media usually form very unstable gels which break down prematurely. On the other hand, gelling agents which form stable, moisture resistant gelled hydrocarbons usually have been incapable of providing the rapid gelling rates required to meet the exigencies of wartime use thereof.

A primary object of this invention is to provide a gelling agent which is effective in small amounts for the gelling of petroleum gasolines, aviation gasoline, kerosene, diesel fuels, and jet fuels at ambient temperatures to form stable gels suitable for use as military incendiaries. Another object of the invention is to gel hydrocarbons at relatively low concentrations and at relatively rapid gelling rates to gels having suitable viscosity, which suitable viscosity is maintained upon aging under variable atmospheric conditions. Still another object of the invention is to provide a method for producing a gelling agent which promotes gelling, in short periods of time, of a wide range of hydrocarbon solvents at ordinary temperatures to form incendiary gels particularly suited for military uses. An additional object is to provide a gelling agent having a gelling rate which is relatively insensitive to temperature. Further objects will appear from the detailed description of the illustrative embodiments of the invention set out hereinafter.

My preferred gelling agent consists of a mixture of isomeric basic aluminum octanoate soaps, defined hereinbelow, in close association with sorbed hydrocarbon oils of lubricating oil viscosity and boiling range; that is,

2

viscosity of from about 100 seconds to 1500 seconds at 100° F. (Saybolt Universal) and initial boiling point above about 575° F. Light hydrocarbon oils are not suitable as presolventing oils. Thus a mineral seal oil having a viscosity of about 50 seconds at 100° F. (Saybolt Universal) when used to presolvent aluminum isoctanoate gelling agent failed to improve the gelation rate of a synthetic gasoline. This failure may have been due to the low boiling range of the mineral seal oil which was from about 500° F. to about 700° F. at atmospheric pressure. The sorbed hydrocarbon oils should be of higher average molecular weight than the liquid hydrocarbons to be gelled by my improved gelling agent. I have discovered that the sorption of the heavy hydrocarbon oils in amounts within the range of about 2.0 percent to about 25 percent, preferably from about 5 percent to about 15 percent, by weight based on the weight of the octanoic acid equivalent of the basic aluminum octanoate soap, increases very substantially the gelation rate of liquid hydrocarbons, particularly when the basic aluminum octanoate gelling agent is used at concentrations below about 6 percent, if the sorption of the oil is concomitant with the precipitation of the basic aluminum octanoate sorbant.

Briefly, the preparation of my preferred gelling agent involves a series of reactions which includes as an initial step of the process, the production of branched chain heptenes by reacting a hydrocarbon stream containing a mixture of propylene and butylenes in the presence of an acid type catalyst such as supported phosphoric acid. The reaction product is fractionated to obtain a fraction consisting essentially of a mixture of branched chain heptenes which are reacted in a second conversion stage with hydrogen and carbon monoxide in the presence of a cobalt-containing catalyst to produce a mixture of iso-octyl aldehydes, i. e., by the well-known oxo process. The iso-octyl aldehyde product is fractionated to obtain a C<sub>8</sub> aldehyde-C<sub>8</sub> alcohol fraction which is then hydrogenated in the presence of a cobalt or nickel catalyst to obtain an iso-octyl alcohol product which product may be fractionated to remove therefrom substantially all components higher boiling and lower boiling than iso-octyl alcohols. The iso-octyl alcohol fraction is converted to the alkali metal soap of the corresponding acids by fusion with an alkali metal hydroxide.

In preparing my improved gelling agent an aqueous solution of the alkali metal soap, such as sodium iso-octanoate soap, and containing sufficient free alkali metal hydroxide, i. e., sodium hydroxide, to form basic aluminum isoctanoates, defined hereinbelow, when contacted with an aqueous solution of an inorganic aluminum salt, such as an aqueous solution of aluminum chloride, is agitated in the presence of a lubricating type petroleum oil to produce an emulsion of the oil in the basic solution of sodium isoctanoate. The aqueous solution of the aluminum salt is then added to the emulsion to produce concomitant precipitation of the branched chain basic aluminum isoctanoate and sorption of the oil therewith. If desired 2-ethylhexanoic acid or an aqueous solution of an alkali metal soap of 2-ethylhexanoic acid may be added to the aqueous solution of alkali metal isoctanoate prior to emulsification of the oil therein, thus providing 2-ethylhexanoate radicals in the improved gelling agent. I also have discovered that sorption of the oil by basic aluminum 2-ethylhexanoate per se from an emulsion of the oil in an aqueous solution of alkali metal 2-ethylhexanoate improves the gelation rate of the 2-ethylhexanoate gelling agent. Presolvement of soap containing 2-ethylhexanoate radicals and isoctanoate radicals with heavy hydrocarbon oils defined above results in marked improvement of gelation time of such soap.

The precipitated soaps are washed free of inorganic salts

and dried, preferably in two steps with an intermediate comminuting step such as grinding. If desired the comminuting step may be carried out in the presence of a small amount of silica aerogel anti-agglomerant or separating agent, that is from about 1.0 percent to about 5 percent based on the weight of soap, to facilitate reduction of the product to a powder and to prevent agglomeration of the finished soap in storage.

More specifically, my improved gelling agents are produced by precipitating branched chain basic aluminum octanoates from basic aqueous solutions of branched chain alkali metal octanoates, said aqueous solutions having emulsified therein a solvating hydrocarbon oil in amount sufficient to provide from about 2 percent to about 25 percent of said oil based on the octanoic acid content of the soap.

In producing the heptene polymer primary intermediate to obtain the isoctanoate component of my improved gelling agent the feed to the polymerization reactor contains from about 30 percent to about 60 percent mixed propylene and butylenes. The mol ratio of propylene to total  $C_3=$  and  $C_4=$  olefins may be varied from about 0.2 to 0.65 with optimum yields of heptenes being obtained at mol ratios of 0.3 to 0.4. It was found that the composition of the branched heptenes did not change appreciably when operating conditions were varied within these ranges. A typical polymer, obtained by polymerizing a  $C_3=$  plus  $C_4=$  stream at a temperature of 385° F., and a pressure of 1200 pounds per square inch in the presence of phosphoric acid catalyst at a conversion of 93 percent, was found to contain in the rough heptene cut, 1 percent hexenes, 89 percent branched chain heptenes, and 10 percent octenes. The analysis of the heptene fraction obtained by the refractionation of the rough cut is shown in Table 1, the analysis being based on temperature and refractive index relations of the various fractions. The heptene cut obtained upon refractionation was used as feed to the oxo process described below.

TABLE 1

Olefin composition:  $C_7$  oxoation feed

| Feed: Parts/1,000 | Component  | Type |
|-------------------|------------|------|
| 12                | 3,3 DMP-1  | G    |
|                   | 4,4 DMP-2  | G    |
| 24                | 2,2 DMP    | F    |
|                   | 2,4 DMP    | E    |
| 47                | 3,4 DMP-1  | B    |
|                   | 2,4 DMP-1  | E    |
| 165               | 2,4 DMP-2  | E    |
|                   | 2,3 DMP-1  | B    |
| 106               | 3,4 DMP-2  | B    |
|                   | 4 MH-2     | C    |
|                   | 2 MH-3     | A    |
|                   | 2 MH-1     | C    |
| 70                | 3 M 2 EB-1 | B    |
| 70                | 2 MH-1     | A    |
|                   | 3 EP-1     | D    |
|                   | 2 EP-1     | C    |
| 259               | 3 MH-2     | C    |
|                   | 3 MH-3     | C    |
|                   | 2 MH-2     | A    |
| 247               | 2,3 DMP-2  | B    |
| 1,000             |            |      |



The above analysis indicates the absence of n-heptenes in the  $C_7$  olefin polymer fraction. The generally accepted mechanism of propylene-butene polymerization in the presence of acid type catalyst is in accord with the conclusion that essentially no straight chain, i. e., n-heptenes, are formed. I have found less than about 1.0 percent normal heptenes in the  $C_7$  olefin fraction subjected to the oxoation process to obtain branched chain  $C_8$  aldehydes and  $C_8$  alcohols for use in obtaining the isoctanoate component of my improved gelling agent. Furthermore, not more than 25 percent to 30 percent of the possible 1.0 percent normal heptenes would oxoate to produce 2-ethylhexylaldehyde which upon hydrogenation would produce 2-ethylhexanol. Thus there is less than about 0.3 percent 2-ethylhexanoic acid in the isoctanoic acid produced from the heptene polymer intermediate.

The mixed  $C_7$  copolymers (branched heptenes) are subjected to the so-called oxo reaction. An equimolar gaseous mixture of hydrogen and carbon monoxide together with the  $C_7$  polymer are contacted in the presence of a cobalt-containing catalyst at temperatures within the range of 300° F. to 400° F., for example 350° F., and at a pressure of about 3000 p. s. i. g. Contact with the catalyst is made at a liquid space velocity within the range of about 0.3 to about 3.0 volumes of liquid per volume of catalyst space per hour. The mol ratio of carbon monoxide to olefin in the feed is within the range of about 1.0 to 1.0 and 3.0 to 1.0. If desired ratios of hydrogen to carbon monoxide as high as 2 to 1 may be used under which conditions larger amounts of  $C_8$  alcohols will be produced in the reaction product which comprises essentially a mixture of branched chain  $C_8$  aldehydes, branched chain  $C_8$  alcohols, unreacted olefins, saturated hydrocarbons and a small amount of heavy polymer. The total reaction product is steam stripped and fractionated to produce a mixture of  $C_8$  alcohols which is essentially free of heavy polymer and which contains only small amounts of non-oxoated hydrocarbon material.

40 The purified oxo product is hydrogenated in the presence of a catalyst such as nickel, cobalt or copper chromite under conditions to selectively reduce the branched  $C_8$  aldehydes of the oxo product mixture to the corresponding branched  $C_8$  alcohols without appreciable reduction of the alcohols to hydrocarbons. For example, the hydrogenation may be carried out at temperatures in the range of about 350° F. to about 500° F., and pressures of 30 to 300 atmospheres in the presence of cobalt catalyst to convert the aldehydes to alcohols. The product is fractionated to obtain a  $C_8$  product consisting essentially of branched chain isomeric octyl alcohols which, for purpose of this specification and claims, I designate as isoctyl alcohol.

45 The purified isoctyl alcohol is converted directly to the alkali metal soaps of the isoctanoic acids corresponding to the mixed isomeric octyl alcohols in the isoctyl alcohol by heating an intimate mixture of the isoctyl alcohol with an alkali metal hydroxide, for example, sodium hydroxide, at temperatures in the range of about 50 600° F.-725° F. The basic aluminum isoctanoate soap is produced by precipitation from aqueous solution of this product with an aqueous solution of an inorganic aluminum salt along with the sorbed oil and, if desired, 2-ethylhexanoate soap as described hereinabove. If desired, the conversion of the isoctyl alcohol to the alkali metal soap may be carried out in the presence of the inert heavy hydrocarbon oil to be sorbed, such as white oil. Water is added to the organic acid-caustic alkali

60 product and the aluminum soap containing the sorbed oil is precipitated therefrom by adding the aqueous solution of aluminum salt such as aluminum chloride.

65 The composition of purified isoctyl alcohols derived from the  $C_7$  copolymer feed of Table 1 was determined by employing the analytical techniques of fractionation,

70

refractometry and infrared spectral analysis of the corresponding octenes derived by dehydration of the purified isooctyl alcohol. Based upon these studies, the estimated composition of the purified isooctyl alcohol is shown in Table 2.

TABLE 2

*Estimated composition of isooctyl alcohol*

| Isomer:                  | Probable range, percent |
|--------------------------|-------------------------|
| 3,4-dimethylhexanol      | 20-30                   |
| 4,5-dimethylhexanol      | 15-25                   |
| 3,5-dimethylhexanol      | 10-15                   |
| 4-methylheptanol         | 10-15                   |
| 3-methylheptanol         | 5-10                    |
| 5-methylheptanol         | 5-10                    |
| 4-ethylhexanol           | 5-10                    |
| 6-methylheptanol         | 5-10                    |
| 3-ethyl-4-methylpentanol | 5-10                    |
| 2,4-dimethylhexanol      | 0-5                     |
| 2,5-dimethylhexanol      | 0-5                     |
| 2-ethyl-4-methylpentanol | 0-5                     |
| 4,4-dimethylhexanol      | 0-5                     |
| 5,5-dimethylhexanol      | 0-5                     |

Certain C<sub>8</sub> alcohol isomers, which are theoretically possible based on the composition of the olefin feed shown in Table 1, were not found in the purified isooctyl alcohol. These isomers may have been lost by fractionation of the isooctyl alcohol. On the other hand, the C<sub>7</sub> olefin precursors of the missing alcohol isomers probably are converted to other C<sub>7</sub> olefin isomers in the oxo reaction by shift of the ethylenic linkage. Thus, for example, no evidence of isopropyl substituent groups in the purified oxo alcohols was found although oxoation of 2-methylhexene-3 should produce, by oxoation and hydrogenation, 2-isopropylpentanol along with 2-ethyl-4-methylpentanol. Likewise, oxoation of 2-methylhexene-2 followed by hydrogenation should yield 2-isopropylpentanol exclusively in the absence of ethylenic linkage isomerization. In like manner oxoation of 2,4-dimethylpentene-2 followed by hydrogenation of the oxoated product should yield 2-isopropyl-3-methylbutanol but with shift of the ethylenic linkage to the 1-position the alcohol product would be 3,5-dimethylhexanol. This branched chain alcohol is present in considerable quantity in the purified C<sub>8</sub> alcohol mixture. Other evidence supports the conclusion that there is extensive isomerization of ethylenic linkage of the olefins in the oxo reaction. For example, it was found that the 247 parts of 2,3-dimethylpentene-2 per 1000 parts of the mixed isomeric C<sub>7</sub> olefins of Table 1 are reduced to only 16 parts by successive passes through the oxo reaction zone, a reduction of about 93 percent. A substantially pure 2,3-dimethylpentene-2 responds to oxoation to the extent of about 70 percent, indicating that according to the accepted theory an ethylenic linkage joining two tertiary carbon atoms will respond to oxoation if, in such oxoation process the ethylenic linkage shifts to a more favorable position. Therefore, a shift of the ethylenic linkage of 2,3-dimethylpentene-2 to the 1-position would produce, by oxoation and reduction, 3,4-dimethylhexanol. It is believed that such shift accounts for a major part of the relatively large amount of 3,4-dimethylhexanol in the purified C<sub>8</sub> alcohol fraction. On the other hand, isomerization of alkyl substituent groups per se in the mixture of isomeric heptenes, which isomerization would result in the alteration of the carbon to carbon structure of the alkyl groups, does not take place in the oxoation stage or in any other stage of the process to which the heptenes and intermediates derived therefrom are subjected in producing the isooctanoate component of my novel gelling agent.

There is less than about 0.3 percent of 2-ethylhexyl alcohol in the purified oxo alcohols. The presence of less than about 0.3 percent of 2-ethylhexyl alcohol in the isooctyl mixture is explained on the basis that this octyl alcohol is derived from only normal straight heptenes

and, as stated above, the heptene polymer mixture contains less than about 1.0 normal straight chain heptenes and the isooctanols contain less than about 0.3 percent 2-ethylhexanol.

Examination of Table 2 indicates that at least 90 percent of the total isomeric C<sub>8</sub> alcohols in the purified oxo alcohol are methyl substituted of which at least 50 percent are dimethyl hexanols and not more than 25 percent of the C<sub>8</sub> alcohols are ethyl substituted, and the C<sub>8</sub> alcohols contain less than about 0.3 percent 2-ethylhexanol. Thus, for purpose of definition in this specification and the claims supported thereby, I use the term isooctanoate to designate the product consisting of mixed branched chain isomeric octanoates which are derived from the isomeric octyl alcohols, that is, the purified C<sub>8</sub> alcohol fraction, and the "isooctanoate" is defined as a soap of isomeric branched chain octanoic acids which acids are at least 90 percent methyl substituted of which at least 50 percent are dimethylhexanoic acids and which acids are not more than 25 percent ethyl substituted and contain less than about 0.3 percent of 2-ethylhexanoic acids, said isomeric branched chain octanoic acids being further characterized by having not more than seven and not less than five carbon atoms in a straight chain.

In the preferred method of drying the basic aluminum octanoate soap containing sorbed oil, the precipitated soap is dehydrated until the moisture content is between about 1.0 percent and 3.0 percent, for example about 1.5 percent. This is accomplished by heating the soap in an oven at about 140°-150° F., for 10 to 18 hours. The soap is then pre-ground to particle size of about 4 mesh and is mixed with about 1 to 5 percent by weight of an inert powder such as a silica aerogel as a separating agent to facilitate final comminution and to reduce the tendency of the final powdered soap to pack. The soap is then reduced to powder form by grinding or other comminuting means after which it is heated for several hours at about 212° F., to reduce the moisture content to the range of 0.2 to about 0.5 weight percent.

The oil presolivated soaps prepared according to the above procedure produce stable gels which in general are insensitive to atmospheric moisture. As indicated in Tables 3 to 7 inclusive, the moisture sensitivity of the soaps was determined. This was accomplished by subjecting the dehydrated soaps to atmospheric conditions of 80 percent relative humidity at 80° F. In this test, the soap, dispersed in thin layers, is subjected to the humid atmosphere for a period of one quarter hour. Such exposure increases the moisture content of the presolivated soap and in general increases the rate of curing of the gels produced from the soap without effecting substantially the stability of the hydrocarbon gels. The characteristic property of accelerating the curing rate without deleterious effect on the stability of the hydrocarbon gel is not common to conventional aluminum soap gelling agents. Thus Napalm is adversely affected by exposure to a highly humid atmosphere, hydrocarbon gels produced from Napalm, so exposed, producing much less stable gels than non-exposed Napalm.

In determining the moisture content of the aluminum soap the benzene azeotrope method is used, that is, essentially the A. S. T. M. Method D-95-46 except that a one-liter flask heated by an electrical heating mantle and containing 500 ml. of benzene solvent is used.

The preparation of the sodium isooctanoate is described below and the preparation of a representative basic aluminum isooctanoate oil-containing soap gelling agent and the preparation of oil-containing basic aluminum 2-ethylhexanoate soap gelling agent according to my invention are described in Examples I and II respectively.

#### SODIUM ISOCTANOATE SOLUTION

A solution of 74.0 weight percent of rayon grade sodium was preheated and pumped at an average rate of 4.5 pounds per hour into the bottom of a cylindrical reaction vessel at about 685° F. The reactor was fitted

with a stirrer and baffles to provide agitation. Oxo process isoctyl alcohol (B. P. 181° C.—192.5° C., N<sub>D</sub> 1.4305, Sp. Gr. 0.833) preheated to about 685° F. was pumped into the bottom of the reactor through a separate inlet at an average rate of 9.3 pounds per hour, reactor temperature being maintained at about 720° F. Oxidation of the alcohol took place with evolution of hydrogen at the rate of about 55 cubic feet per hour. This gas was vented at such a rate as to maintain a pressure of about 210 p. s. i. g. on the reactor and solution vessel. The sodium isoctanoate, excess sodium hydroxide, and trace of unreacted alcohol passed through an overflow line at the top of the reactor into a solution vessel held at a temperature of about 410° F. where water was added at the rate of about 29 pounds per hour to dissolve the soap and excess caustic. Unreacted alcohol was flashed off with steam from the top of the solution vessel to a separator where it was recovered at a rate of about 0.3 pound per hour. Over a twenty-one hour period, 194.8 pounds of the isoctyl alcohol was fed to the reactor and there was recovered sodium isoctanoate soap equivalent to 187.9 pounds of isoctyl alcohol corresponding to a yield of 96.2 percent, along with 6.9 pounds of unconverted isoctyl alcohol. An aqueous soap solution was withdrawn from the bottom of the solution vessel and cooled. This solution had an average analysis corresponding to the following:

|                                 | Weight percent |
|---------------------------------|----------------|
| Sodium isoctanoate              | 45.8           |
| Water                           | 51.7           |
| NaOH                            | 2.0            |
| Na <sub>2</sub> CO <sub>3</sub> | 0.5            |
| Free isoctyl alcohol            | Trace          |
|                                 | 100.0          |

EXAMPLE I.—OIL-CONTAINING BASIC ALUMINUM ISOCTANOATE SOAP

To 3380 parts by weight of water in a precipitation vessel was added 17.6 parts by weight of NaOH. To this alkali solution was added 1460 parts by weight of sodium isoctanoate solution containing 462 parts by weight of sodium isoctanoate and 149 parts by weight of free NaOH. There was then added slowly, with agitation of the sodium isoctanoate solution, 60 parts of a medicinal heavy grade petroleum white oil having a viscosity of 360 seconds at 100° F. (Saybolt Universal) corresponding to 20 percent of oil based on the isoctanoic acid in the solution. Stirring of the solution was continued until the oil was completely emulsified to give a creamy uniform emulsion. While agitating this emulsion 845 parts by weight of 32° Bé. aluminum chloride solution dissolved in 1220 parts by weight of water was added. The pH of the basic sodium isoctanoate solution before aluminum chloride addition was about 14. Precipitation started at a pH of about 9.5. The final pH was about 3.5 at which point there remained no emulsified oil in the supernatant liquid. The precipitated basic aluminum isoctanoate containing sorbed oil was filtered, washed free of chloride, rough ground and dried for about 18 hours at about 150° F. to a moisture content of 0.7 percent. The partially dried soap was then thoroughly mixed with 5 percent (by weight) of a silica aerogel (Santocel) and reground to a powder of a fineness corresponding to about 75 percent passing a 100 mesh screen and the comminuted product was then heated for about three hours at 210°–212° F. The oil-containing basic aluminum isoctanoate soaps used in obtaining the results given in Tables 4, 5, and 6 below were prepared according to the above procedure, using the appropriate amount of oil in the emulsification step to give the indicated sorbed oil content in the specific soaps. The soaps described in Table 3 (oil content zero) were

prepared in like manner except that no oil was emulsified in the basic sodium isoctanoate solution.

EXAMPLE II.—OIL-CONTAINING BASIC ALUMINUM 2-ETHYLHEXANOATE SOAP

To 2000 grams of water was added 82 grams of NaOH and 200 grams of 2-ethylhexanoic acid. The mixture was stirred to obtain complete solution of the 2-ethylhexanoic acid and then 40 grams of petroleum medicinal white oil (of the same grade as used in Example I) was emulsified in the basic aqueous solution of sodium 2-ethylhexanoate. The solution before oil addition had a pH of 12+. To the emulsion was added slowly, a mixture of 330 ml. of AlCl<sub>3</sub> solution (32° Bé.) in 370 grams of water. The pH dropped to about 3.5 during the precipitation of the basic aluminum 2-ethylhexanoate containing the sorbed oil, i. e., about 20 percent oil by weight, based on the 2-ethylhexanoic acid. The precipitate was filtered and washed free of inorganic salt and dried for fifteen hours at 150° F. after which it was ground to a powder corresponding to about 75 percent passing through a 100 mesh screen. It was then dried for an additional six hours at about 140° F. This soap was used to obtain the data given for oil-containing basic aluminum 2-ethylhexanoate in Table 7. Data given in Table 7 for oil-free basic aluminum 2-ethylhexanoate soap were obtained from 2-ethylhexanoate soap prepared in like manner except that oil was not emulsified in the aqueous solution of basic aluminum 2-ethylhexanoate.

In using the gelling agents produced according to the foregoing procedures, a quantity of the agent is added to the hydrocarbon fuel and stirred at ambient temperature. Between about 0.5 and about 6.0 weight percent, preferably between about 1.0 and 4.0 weight percent of the precipitated basic aluminum octanoates, the octanoate radicals of which consist essentially of branched chain isoctanoate radicals and/or 2-ethylhexanoate radicals produce, with the sorbed oil, the superior gels. The novel gelling agents are particularly effective when used at relatively low concentrations, that is, about 1.5 weight percent to about 5 weight percent in gelling gasolines, kerosenes, diesel fuels, jet fuels, and the like to relatively high gel viscosity in a shorter period of time than oil-free soaps and the gels mature more rapidly than gels produced with oil-free soaps.

Gelation begins immediately when the agent and liquid are stirred at ambient temperatures. The extent of initial gelation is a measure of the gelling properties and is determined by a standard test described hereinafter as the "Vortex Time," that is, the time necessary to obtain a specific diminution of the amplitude of a vortex in a mass stirred under defined conditions. This "Vortex Time" is a measure of the rate at which a gelling agent causes a hydrocarbon solvent to thicken. A Vortex Time of about 10 minutes or less, in the production of gels having the higher consistency range described hereinbelow, is desired. This is realized with my improved gelation agent at the 4 percent concentration level. Even at lower concentrations of my improved gelling agent which give Gardner Load values in the lower viscosity range described below, Vortex Times lower than 10 are possible.

For general laboratory testing of gelling agents a quantity of the hydrocarbon solvent is introduced into a square-type pint Mason jar having dimensions approximately 3 inches by 3 inches by 5 inches deep. A total weight of 200 grams of solvent and gelling agent is employed. For example, if 4 weight percent gel is to be prepared, 8 grams of the gelling agent will be added to 192 grams of the solvent.

A glass stirring rod is employed which is about  $\frac{3}{8}$  inch in diameter with four vanes,  $\frac{1}{8}$  by  $\frac{1}{8}$  by  $\frac{1}{8}$  inch, set at right angles and having faces parallel to the axis of the rod. The stirrer is mounted within the jar with the bottom of the stirrer  $\frac{1}{2}$  inch above the bottom of

the jar. A reference mark is made on the glass rod one centimeter below the surface of the test solvent.

The stirring speed is adjusted to  $300 \pm 10$  R. P. M. and the temperature of the solution is controlled at some standardized temperature. Examples shown below in Tables 3 to 7 inclusive were carried out at  $77^{\circ}$  F. and  $35^{\circ}$  F. The time elapsed between addition of the gelling agent sample and immersion of the reference mark by the rising vortex is recorded as the "Vortex Time." The gel continues to cure for from 6 hours to about a day without stirring after the initial gelation occurs, as measured by the "Vortex Time."

The properties of the final gel are measured by the "Gardner Load," which is a measure of the viscosity and indicates the consistency and when the "Gardner Load" values are determined at time intervals following initial gelation the values obtained indicate the stability of the cured hydrocarbon gel with respect to consistency. It is determined in a Gardner Mobilometer, an apparatus described in "Physical and Chemical Examination of Paints, Varnishes, Lacquers and Colors," 10th edition (May 1946) by Henry A. Gardner and G. G. Sward, distributed by Henry A. Gardner Laboratory, Inc., Bethesda, Maryland. The test is ordinarily made at 24 or 48 hours after initial gelling has taken place and the values are in terms of grams per 100 seconds. In general, a Gardner Load in the range of about 100 to about 225 grams designates a desirable consistency for portable flame thrower service whereas a load of about 350 to about 650 grams indicates a suitable consistency for other military incendiary purposes. Ordinarily the load should remain below about 650 grams if the gel is to have the desired splattering, cohesion and burning properties. My improved oil-containing basic aluminum octanoate gelling agent produces, with gasolines, a product which is a 35 stringy material having high splattering and good cohesion and burning properties when dispersed by flame-thrower apparatus.

The instrument used in the Gardner tests consists essentially of a cylinder supported on a base plate, a plunger or piston, and a collar to support the plunger. The cylinder is 8.0 inches deep and 1.538 inches in diameter. The plunger consists of a disc 1.500 inches in diameter with four perforations 0.250 inch in diameter and a weight pan or holder supported by the upper end of a tube or rod fixed at its lower end to the disc. The weight of the moving system which includes the disc, connecting rod or tube, and the weight support is 100 grams.

To make the test, the cylinder is filled to a depth of 20 centimeters with the gel to be tested and is leveled by means of adjusting screws. The disc end of the plunger is then introduced into the cylinder with the connecting

noting two successive loads in grams corresponding to more than and less than 100 seconds travel, the load required to give a time fall of 100 seconds being obtained by linear interpolation from these two readings.

The desirable properties of the oil-sorbed basic aluminum octanoate soaps as gelling agents in standard test solvent have been compared with the properties of the corresponding oil-free basic aluminum octanoates in Tables 3 to 7 inclusive hereinbelow. The formulation of the standard "test solvent" used in evaluating the gelling agents conforms to Military Standard MS602 (October 22, 1951) and has the following composition:

|    |             | Weight per cent |
|----|-------------|-----------------|
| 15 | N-heptane   | 57              |
|    | Benzene     | 18              |
|    | Cyclohexane | 20              |
|    | Isooctane   | 5               |

TABLE 3  
Gelling properties of basic aluminum isoctanoate soap containing no sorbed oil

|    | Evaluation                          | 1   | 2    | 3   | 4    | 5   | 6    |
|----|-------------------------------------|-----|------|-----|------|-----|------|
| 25 | Exposure to Moist Air, hrs.         | 0   | 0.25 | 0   | 0.25 | 0   | 0.25 |
|    | Moisture in Final Soap, wt. Percent | 0.4 | 1.3  | 0.4 | 1.3  | 0.4 | 1.4  |
|    | Wt. Percent Soap in Gel             | 1.5 | 1.5  | 2.0 | 2.0  | 4.0 | 4.0  |
|    | At $77^{\circ}$ F.:                 |     |      |     |      |     |      |
|    | Vortex Time, min.                   | 75  | 40   | 75  | 28   | 2.4 | 3.1  |
| 30 | Gardner Load, g./100 sec.           |     |      |     |      |     |      |
|    | at 24 hrs.                          | 150 | 150  | 225 | 210  | 620 | 515  |
|    | at 48 hrs.                          | 155 | 145  | 190 | 200  | 550 | 490  |
|    | at 168 hrs.                         | 155 | 105  | 190 | 175  | 625 | 490  |

<sup>1</sup> Humidity test consists of submitting soap to relative humidity of 80 percent at  $80^{\circ}$  F. for a period of  $\frac{1}{4}$  hr.

The basic aluminum isoctanoate gelling agent used for experiments 1 to 6 inclusive in Table 3 contained no sorbed oil. The gels described in Table 3 are typical laboratory-prepared gels produced by oil-free isoctanoate gelling agent, that is, gelling agents having relatively low gelling rates at soap concentrations of 2 percent or less. The gelling rates of the non-presolivated soaps may also be improved by heat treatment as taught and claimed in copending application, Serial No. 339,504, filed March 2, 45 1953, entitled "Rapid Gelling Basic Aluminum Soaps."

In Table 4 below are shown the gelling rates of basic aluminum isoctanoate soap containing different amounts of sorbed medicinal grade heavy white oil. This oil had a viscosity of about 350 seconds at  $100^{\circ}$  F. (Saybolt Universal). Viscosity-time performance of the hydrocarbon gels prepared from synthetic gasoline (standard test solvent) is also included in the table.

TABLE 4  
Gelling properties of basic aluminum isoctanoate soap containing sorbed white oil

| Evaluation                          | 7   | 8    | 9   | 10   | 11   | 12   | 13   | 14   | 15   | 16   | 17   | 18   |
|-------------------------------------|-----|------|-----|------|------|------|------|------|------|------|------|------|
| Wt. Percent Oil in Soap             | 2.0 | 2.0  | 5.0 | 5.0  | 10.0 | 10.0 | 10.0 | 10.0 | 15.0 | 15.0 | 15.0 | 15.0 |
| Exposure to Moist Air, hrs.         | 0   | 0.25 | 0   | 0.25 | 0    | 0.25 | 0    | 0.25 | 0    | 0.25 | 0    | 0.25 |
| Moisture in Final Soap, wt. Percent | 0.4 | 1.4  | 0.6 | 1.4  | 0.3  | 1.4  | 0.3  | 1.4  | 0.3  | 1.4  | 0.3  | 1.4  |
| Wt. Percent Soap in Gel             | 2.0 | 2.0  | 2.0 | 2.0  | 2.0  | 2.0  | 4.0  | 4.0  | 2.0  | 2.0  | 4.0  | 4.0  |
| AT $77^{\circ}$ F.:                 |     |      |     |      |      |      |      |      |      |      |      |      |
| Vortex Time, min.                   | 71  | 22   | 41  | 19   | 5.5  | 7.0  | 1.7  | 2.4  | 3.1  | 4.1  | 1.3  | 1.8  |
| Gardner Load, g./100 sec.           |     |      |     |      |      |      |      |      |      |      |      |      |
| at 24 hrs.                          | 225 | 200  | 240 | 210  | 295  | 225  | 705  | 645  | 280  | 220  | 685  | 540  |
| at 48 hrs.                          | 190 | 190  | 220 | 205  | 265  | 210  | 705  | 540  | 265  | 200  | 600  | 505  |
| at 168 hrs.                         | 180 | 180  | 180 | 150  | 220  | 195  | 630  | 600  | 250  | 180  | 685  | 450  |

tube aligned by a collar. The time required for two marks 10 centimeters apart on the stem of the plunger to pass through the collar is then recorded. The pair of marks are located so that they pass through the collar of the bracket as the disc passes through the mid-portion of the cylinder. Thus the plunger is in motion both at the beginning and at the end of the test interval. In reporting results, the "Gardner Load" is determined by

70 It will be noted (Table 4) that the gelling rate increases as the percent of sorbed oil in the isoctanoate gelling agent is increased, the amount of soap used remaining constant. Comparing Evaluations 3 and 4 of Table 3 with Evaluations 11 and 12 of Table 4, it is seen that the Vortex Time has been greatly reduced by the presence of 10 percent sorbed heavy white oil. In general, higher viscosities of the gels with a given concentra-

tion of gelling agent are realized with increasing amounts of sorbed oil.

In Table 5 is shown the performance of aluminum isoctanoate gelling agent having sorbed therewith two different oils of approximately the same viscosity range,

duces fast-curing stable gels with liquid hydrocarbons. The data also indicate the wide range of oils with respect to viscosity, which can be used to improve the gelling rate by sorbing the same with isoctanoate soap gelling agent.

TABLE 7

*Gelling performance of basic aluminum 2-ethylhexanoate soap with and without sorbed white oil*

| Evaluation                  | 43  | 44   | 45  | 46   | 47  | 48   | 49  | 50   |
|-----------------------------|-----|------|-----|------|-----|------|-----|------|
| Wt. Percent Oil in Soap     | 20  | 20   | 20  | 20   | 0   | 0    | 0   | 0    |
| Exposure to Moist Air, hrs. | 0   | 0.25 | 0   | 0.25 | 0   | 0.25 | 0   | 0.25 |
| Wt. Percent Soap in Gel     | 1.7 | 1.7  | 3.3 | 3.3  | 2   | 2    | 4   | 4    |
| At 77° F.:                  |     |      |     |      |     |      |     |      |
| Vortex Time, min.           | 27  | 29   | 1.2 | 1.6  | 78  | 62   | 5.8 | 5.3  |
| Gardner Load, g./100 sec.—  |     |      |     |      |     |      |     |      |
| at 24 hrs.                  | 100 | 60   | 355 | 425  | 90  | 105  | 350 | 345  |
| at 168 hrs.                 | 255 | 245  | 460 | 520  | 215 | 195  | 515 | 510  |

the blended oil being a non-extracted oil and the other oil being a conventional solvent extracted lubricating oil.

In Table 7, a comparison of the gelling properties of oil-free basic aluminum 2-ethylhexanoate soap is made

TABLE 5

*Gelling performance of aluminum isoctanoate soap containing 12.5% sorbed heavy oils*

| Evaluation                          | High Flash Blended Petroleum Oil <sup>1</sup> |      |     |      |     |      | SAE 20 (Solvent Extracted) |      |     |      |     |      |
|-------------------------------------|-----------------------------------------------|------|-----|------|-----|------|----------------------------|------|-----|------|-----|------|
|                                     | 19                                            | 20   | 21  | 22   | 23  | 24   | 25                         | 26   | 27  | 28   | 29  | 30   |
| Exposure to Moist Air, hrs.         | 0                                             | 0.25 | 0   | 0.25 | 0   | 0.25 | 0                          | 0.25 | 0   | 0.25 | 0   | 0.25 |
| Moisture in Final Soap, Wt. Percent | 0.4                                           | 1.4  | 0.4 | 1.4  | 0.4 | 1.4  | 0.2                        | 1.2  | 0.2 | 1.2  | 0.2 | 1.2  |
| Wt. Percent Soap in Gel             | 1.4                                           | 1.4  | 1.8 | 1.8  | 3.6 | 3.6  | 1.4                        | 1.4  | 1.8 | 1.8  | 3.6 | 3.6  |
| At 77° F.:                          |                                               |      |     |      |     |      |                            |      |     |      |     |      |
| Vortex Time, min.                   | 9.0                                           | 11   | 7.0 | 7.1  | 2.1 | 2.4  | 11                         | 21   | 7.8 | 15   | 2.2 | 2.4  |
| Gardner Load, g./100 sec.—          |                                               |      |     |      |     |      |                            |      |     |      |     |      |
| at 24 hrs.                          | 175                                           | 130  | 205 | 175  | 555 | 455  | 205                        | 180  | 240 | 190  | 620 | 465  |
| at 48 hrs.                          | 140                                           | 120  | 190 | 160  | 465 | 390  | 165                        | 145  | 225 | 180  | 540 | 450  |
| at 168 hrs.                         | 175                                           | 110  | 180 | 160  | 450 | 370  | 175                        | 150  | 215 | 170  | 560 | 410  |

<sup>1</sup> Viscosity at 100° F., 300 (S.S.U.)

Referring to Table 5 above, it is seen that basic aluminum isoctanoate soaps containing 12.5 percent by weight of sorbed, relatively high boiling hydrocarbon oils are quite effective at low soap concentrations for increasing the rate of gelation and in the production of relatively stable gels at these low concentrations. The data indicate that it is not necessary to use, as sorption oils in my improved gelling agent, highly refined oils such as white oils or solvent extracted oils but that oils which have not undergone acid treatment or solvent extraction are suitable.

The performance of aluminum isoctanoate gelling agent containing sorbed, solvent extracted lubricating oils of S. A. E. 10 and S. A. E. 50 grade is shown in Table 6.

40 with such soap containing 20 weight percent of heavy grade medicinal white oil (described above). Although the effect of the sorbed oil in regard to gelation properties is less marked with basic aluminum 2-ethylhexanoate soap than is the case with oil-sorbed aluminum isoctanoate soap, there is a marked increase in gelation rate, that is, approximately a fourfold increase in the rate at the 4 percent soap concentration level.

50 The above data indicate that my improved basic aluminum octanoate soaps containing sorbed oil to the extent of from about 2.0 weight percent to about 25 weight percent based on the octanoic acid equivalent of the octanoate content of said soap are effective in increasing the gelling rate and in the production of rapid curing of stable

TABLE 6

*Gelling performance of aluminum isoctanoate soap containing sorbed lubricating oils*

| Evaluation                         | S. A. E. 10 (Solvent Extracted) <sup>1</sup> |      |     |      |     |      | S. A. E. 50 (Solvent Extracted) <sup>2</sup> |      |      |      |      |      |
|------------------------------------|----------------------------------------------|------|-----|------|-----|------|----------------------------------------------|------|------|------|------|------|
|                                    | 31                                           | 32   | 33  | 34   | 35  | 36   | 37                                           | 38   | 39   | 40   | 41   | 42   |
| Wt. percent Oil in Soap            | 20                                           | 20   | 20  | 20   | 20  | 20   | 12.5                                         | 12.5 | 12.5 | 12.5 | 12.5 | 12.5 |
| Exposure to Moist Atmosphere, hrs. | 0                                            | 0.25 | 0   | 0.25 | 0   | 0.25 | 0                                            | 0.25 | 0    | 0.25 | 0    | 0.25 |
| Moisture in Final Soap             | 0.4                                          | 1.0  | 0.4 | 1.0  | 0.4 | 1.0  | 0.3                                          | 1.1  | 0.3  | 1.1  | 0.3  | 1.1  |
| Wt. percent Soap in Gel            | 1.5                                          | 1.5  | 2.0 | 2.0  | 4.0 | 4.0  | 1.4                                          | 1.4  | 1.8  | 1.8  | 3.6  | 3.6  |
| At 77° F.:                         |                                              |      |     |      |     |      |                                              |      |      |      |      |      |
| Vortex Time, min.                  | 8.2                                          | 14   | 5.0 | 11   | 2.5 | 3.3  | 32                                           | 26   | 16   | 18   | 0.9  | 1.5  |
| Gardner Load, g./100 sec.—         |                                              |      |     |      |     |      |                                              |      |      |      |      |      |
| at 24 hrs.                         | 195                                          | 185  | 265 | 220  | 600 | 495  | 165                                          | 170  | 230  | 205  | 570  | 520  |
| at 48 hrs.                         | 185                                          | 175  | 245 | 215  | 600 | 520  | 185                                          | 160  | 230  | 195  | 550  | 490  |
| at 168 hrs.                        | 155                                          | 160  | 240 | 220  | 580 | 500  | 165                                          | 145  | 215  | 190  | 505  | 480  |

<sup>1</sup> Viscosity 165 seconds at 100° F. (Saybolt Universal).

<sup>2</sup> Viscosity 1462 seconds at 100° F. (Saybolt Universal).

The performance data indicate that a hydrocarbon oil as viscous as S. A. E. 50 grade when sorbed by isoctanoate soap is effective in reducing the vortex time and pro-

50 gels of liquid hydrocarbons when the presorbed soap is used in a concentration of from about 0.5 percent to about 6 percent in said hydrocarbon oils.

I claim:

1. The method of making an agent for gelling a hydrocarbon boiling in the range of about 100 to 600° F., which method comprises intimately mixing an inorganic, water-soluble, aluminum salt with a dilute aqueous solution of alkali metal branched chain octanoate and alkali metal hydroxide in the presence of a heavy hydrocarbon oil having a Saybolt Universal viscosity in the range of about 100 to 1500 seconds at 100° F. and being of higher boiling range than the hydrocarbon to be gelled, the amount of said heavy hydrocarbon oil being in the range of about 2 to 25 per cent by weight based on the octanoic acid equivalent of the alkali metal branched chain octanoate in said solution, said heavy hydrocarbon oil being emulsified in aqueous solution during said mixing and sorbed in the water-insoluble basic aluminum branched chain octanoate which is precipitated during said mixing the branches on the branched chain octanoate radicals being selected from the class consisting of methyl and ethyl, washing the precipitated basic aluminum branched chain octanoate soap to free the precipitate of alkali metal and inorganic salt, drying said precipitate to a moisture content of not more than 3 per cent, and grinding the dried basic aluminum branched chain octanoate with the heavy oil sorbed therein.

2. The method of claim 1 wherein the heavy hydrocarbon oil is a white oil.

3. The method of claim 1 wherein the heavy hydrocarbon oil is emulsified in an aqueous solution of sodium branched chain isoctanoate soap and an aqueous aluminum chloride solution is added thereto during the mixing step.

4. The method of claim 1 which includes the step of

mixing about 1 to 5 per cent of a silica aerogel with the oil-sorbed basic aluminum branched chain octanoate prior to a final grinding step.

5. The method of claim 4 which includes the step of heating the oil-sorbed basic aluminum branched chain octanoate after the final grinding step to reduce its moisture content to a range of about .02 to .5 weight per cent.

6. The method of claim 1 wherein the alkali metal branched chain octanoate is sodium isoctanoate.

7. The method of claim 1 wherein the alkali metal branched chain octanoate is sodium 2-ethyl hexanoate.

8. The method of claim 1 wherein the alkali metal branched chain octanoate is a mixture of about 10 to 60 weight per cent of sodium 2-ethyl hexanoate and 90 to 40 weight per cent of sodium isoctanoate.

9. The method of claim 1 wherein the amount of heavy hydrocarbon oil is in the range of about 5 to 20 per cent by weight based on octanoic acid equivalent of the alkali metal branched chain octanoate.

10. The method of claim 1 wherein the inorganic water-soluble aluminum salt is aluminum chloride.

25

30

References Cited in the file of this patent

UNITED STATES PATENTS

|           |                |               |
|-----------|----------------|---------------|
| 2,390,609 | Minich         | Dec. 11, 1945 |
| 2,417,071 | Gebhart et al. | Mar. 11, 1947 |
| 2,582,833 | Hunn           | Jan. 15, 1952 |
| 2,584,041 | Nowak et al.   | Jan. 29, 1952 |
| 2,618,536 | Hunn           | Nov. 18, 1952 |
| 2,628,202 | Allison et al. | Feb. 10, 1953 |
| 2,626,897 | Young et al.   | Jan. 27, 1953 |